

J. L. Tuttle,

Preparing Card-Teeth Wire.

No 15,905.

Patented Oct. 14, 1866.



# UNITED STATES PATENT OFFICE.

JOHN L. TUTTLE, OF NEW YORK, N. Y.

## IMPROVEMENT IN CARD-TEETH FOR MACHINE-CARDS.

Specification forming part of Letters Patent No. 15,905, dated October 14, 1856.

*To all whom it may concern:*

Be it known that I, JOHN L. TUTTLE, of the city, county, and State of New York, have invented certain new and useful Improvements in the Preparation of Steel Wire to be Used for Card or Cylinder Teeth for Working or Cleaning Wool or Cotton; and I do hereby declare the following to be a full, clear, and exact description of the same, reference being had to the accompanying drawings, making a part of this specification, in which—

Figures 1, 2, 3 represent side and back views of the wire. Figs. 4, 5, 6 represent cross-sections through the same. Fig. 7 represents a manner of setting the teeth.

The nature of my invention relates to certain improvements in card-teeth by the preparation of previously-drawn steel wire to be used in cards, clothing, or cylinders for carding wool or cleaning cotton; and it consists in so shaping or flattening round steel wire as that when set in the cards or on cylinders and ground off to make a surface the same operation shall make a point to each tooth, as will be described.

I take round steel wire of suitable size and pass it through between grooved rollers of such form as will flatten it out on one side of its center to nearly a knife-edge, or so that a section through or across such rolled or flattened wire would resemble in appearance a section through a razor-blade. It is immaterial as to the exact form of the back of the wire, but important to have its edge portion flattened to a knife-edge, or nearly so. The wire thus formed may be tinned and then set in a cylinder, as described in the Letters Patent granted to me on the 30th October, 1849.

There is a marked difference between the drawing of steel wire through dies and the flattening or shaping of such wire, as herein set forth, by passing it through between steel or hard rollers after it has been drawn out through the dies. In drawing wire the fiber of the metal follows the direction of the progressive drawings through the dies. I take the wire thus drawn and flatten out one-half of it, or thereabout, bringing it down to a knife-edge, but not a serrated or rough edge, but one perfectly smooth, the fiber being rolled at right angles to its position in the drawn wire; and to keep the wire from undue spread-

ing or from separation of its fiber, I place the rolls in oil, which prevents any tendency of the fibers to part, turn out, or make a rough surface. The opposite side of the wire from a longitudinal line drawn through its center may remain in the form in which it comes from the die; or it may be slightly pressed in toward that part which is flattened out to prevent the fiber from separating laterally.

Fig. 1 represents a side view, and Figs. 2, 3 represent a back view, of the flattened wire, the lower portions being represented as unrolled. Figs. 4, 5, and 6 show the form of the wire in cross-section after it is flattened, all the figures being drawn on an enlarged scale to better represent the form.

When the flattened wire *a a a* is set in the cards, it is cut off in an oblique direction, so as to form a point, *b b b*, next the knife-edge. After the teeth are set in the cards or cylinder, they are ground off on their oblique or inclined ends to "surface" them, (as it is termed,) and this also at the same time produces the points *b*, and saves not only the necessity of file-dressing, but makes a better point and at a better location in the tooth for entering the fiber.

In resharpening the teeth it is only necessary to resurface, one operation completing the whole until the teeth are entirely worn out. This method of preparing the article leaves no feathered or fin edges to catch, hold, or clog the cards with the fiber.

Having thus fully described the nature of my invention and shown how the same may be used, I would state that I am aware that Richd. Kitson, in his patent of November 11, 1851, represents a tooth of soft iron and of small wire with a cross-section resembling the cross-section of my card-teeth. This I do not claim; but

What I do claim as new, and desire to secure by Letters Patent, is—

The making of card-teeth by giving to steel wire the form herein described and substantially in the manner set forth, so that when set and a surface ground on them, the same grinding shall form the sharp points thereon.

J. L. TUTTLE.

Witnesses:

A. B. STOUGHTON,  
E. COHEN.